

1

3,502,580

## GREASE COMPOSITION

Keith Coupland, Hornsea, England, assignor to BP Chemicals (U.K.) Limited, London, England, a British company.  
No Drawing. Filed Oct. 4, 1967, Ser. No. 672,693  
Claims priority, application Great Britain, Oct. 29, 1966,  
48,603/66  
Int. Cl. C10m 7/44  
U.S. Cl. 252—42.1

5 Claims 10

### ABSTRACT OF THE DISCLOSURE

The invention is a grease composition suitable for use under extreme pressure conditions comprising a base fluid, an alkali metal salt of a fatty acid and a tris-(2-chloroalkyl) ester of an oxyacid of phosphorus. 15

The present invention relates to grease compositions suitable for use under extreme pressure conditions. 20

According to the invention, a grease composition suitable for use under extreme pressure conditions comprises a base fluid, an alkali metal salt of a fatty acid and a tris-(2-chloroalkyl) ester of an oxyacid of phosphorus. 25

The base fluid is suitably a hydrocarbon or preferably an ester which may be used as a synthetic lubricant base. Examples include esters of polyhydroxy compounds, such as trimethylol propane tricaprylate, and esters of polycarboxylic acids such as dinonyl sebacate. Other examples are the 2:2:6:6-tetrakis alkyl-cyclohexanone- $\beta$ -propionate, 2:2:5:5-tetrakis alkyl-cyclopentone- $\beta$ -propionate, 2-alkyl-2:6:6-tris-alkyl - cyclohexanone -  $\beta$  - propionate and 2 - alkyl - 2:5:5-tris-alkyl-cyclopentanone- $\beta$ -propionate esters whose use as lubricant bases is disclosed in British patent specification 1,036,692. 30

The alkali metal salt, which is preferably the lithium salt, acts as a thickener and may be, for example, the palmitate, oleate, 12-hydroxystearate or preferably the stearate. It should comprise from 5 to 30% by weight, preferably 10-20% of the composition. 35

Examples of suitable tris-(2-chloroalkyl) esters of the oxyacids of phosphorus are tris-(2-chloroethyl) and tris-(2-chloropropyl) phosphite, and also the corresponding phosphate ester. The concentration of the ester in the composition should be in the range 0.1-5.0% by weight preferably 0.5-2%. 40

The compositions may also contain conventional grease additives such as antioxidants and rust and corrosion inhibitors. 50

The greases may be prepared by heating together the ester lubricant and alkali metal salt while stirring until a clear solution is obtained. The solution is cooled rapidly

2

to give a gel which is "worked" to give the desired grease.

The grease may also conveniently be prepared by generating the alkali metal salt in situ by addition of the fatty acid and saponifying it with alkali metal hydroxide, with the removal of water. The ester of the oxyacid of phosphorus may be included at any stage of manufacture but for convenience and to avoid undesirable interaction at high temperature they are conveniently included at the cold working stage. The cold working procedure involves milling or mixing at high shear rates to give a grease of smooth appearance.

The grease formulations are further illustrated in the following examples.

### EXAMPLE 1

A mixture of lithium stearate (10 parts) and dinonyl sebacate (90 parts) was heated with stirring to 140° C. and held at this temperature for 1 hour. The temperature was then raised to 185° C. and the resulting solution cooled rapidly to give a gel. The cooled gel was worked in a high shear mixer until a grease of smooth appearance resulted. 20

### EXAMPLE 2

The procedure of Example 1 was followed using the same proportions but tris-(2-chloroethyl) phosphite (1 part) was milled in at the cold working stage. 25

### EXAMPLE 3

As for Example 2 substituting tris-(2-chloropropyl) phosphite (1 part) as extreme pressure agent. 30

### EXAMPLE 4

As for Example 1 substituting trimethylol propane tricaprylate as the ester lubricant. 35

### EXAMPLE 5

As for Example 4 with the addition of tris-(2-chloroethyl) phosphite (1 part) as extreme pressure additive. 40

### EXAMPLE 6

As for Example 4 with the addition of tris-(2-chloroethyl) phosphite (1 part) as extreme pressure additive. 45

### EXAMPLE 7

As for Example 1 substituting 2:2:6:6-tetrakis butyl-cyclohexanone-beta-propionate as the ester lubricant. 50

### EXAMPLE 8

As for Example 7 with the addition of tris-(2-chloroethyl) phosphite (1 part) as extreme pressure additive.

The results of extreme pressure tests using the above formulations are indicated in Table 1.

TABLE 1  
10 sec. Wear Scar Diameters (Shell Four Ball Test)  
[10% lithium stearate greases with EP additives at 1% concentration]

| Base Fluid                                           | Example | EP additive (at 1% concentration) | Wear Scar diameter (mm.) |        |         |
|------------------------------------------------------|---------|-----------------------------------|--------------------------|--------|---------|
|                                                      |         |                                   | 50 kg.                   | 75 kg. | 100 kg. |
| Dinonyl sebacate                                     | 1       | None                              | 0.345                    | 2.23   | 2.24    |
|                                                      | 2       | Tris-(2-chloroethyl) phosphite    | 0.324                    | 0.381  | 2.07    |
|                                                      | 3       | Tris-(2-chloropropyl) phosphite   | 0.350                    | -----  | -----   |
| Trimethylol propane tricaprylate                     | 4       | None                              | 0.378                    | 2.06   | 3.29    |
|                                                      | 5       | Tris-(2-chloroethyl) phosphite    | 0.355                    | 0.830  | 2.21    |
|                                                      | 6       | Tris-(2-chloropropyl) phosphite   | 0.359                    | 0.575  | 2.09    |
| 2:2:6:6-tetrakis butyl-cyclohexanone-beta-propionate | 7       | None                              | 0.324                    | 0.506  | 2.23    |
|                                                      | 8       | Tris-(2-chloroethyl) phosphite    | 0.347                    | 0.400  | 1.96    |

## I claim:

1. A grease composition suitable for use under extreme pressure conditions comprising a synthetic base fluid, from 5 to 30% by weight of the composition of a lithium salt of a fatty acid selected from the group consisting of stearic, palmitic, oleic and hydroxystearic and a tris-(2-chloroalkyl) ester of an oxyacid of phosphorus comprising 0.1 to 5.0% by weight of the composition.

2. A grease composition according to claim 1 wherein the base fluid is trimethylol propane tricaprlyate.

3. A grease composition according to claim 1 wherein the base fluid is dinonyl sebacate.

4. A grease composition according to claim 1 wherein the base fluid is selected from 2:2:6:6-tetrakis alkyl-cyclohexanone- $\beta$ -propionate, 2:2:5:5-tetrakis alkyl-cyclopentanone- $\beta$ -propionate, 2-alkyl-2:6:6-tris-alkyl-cyclohexanone- $\beta$ -propionate or 2-alkyl-2:5:5-tris alkyl-cyclopentanone- $\beta$ -propionate.

5. A grease composition according to claim 1 wherein the tris-(2-chloroalkyl) ester of an oxyacid of phosphorus is selected from tris-(2-chloroethyl) phosphite, tris-(2-

chloropropyl) phosphite, tris-(2-chloroethyl) phosphate or tris-(2-chloropropyl) phosphate.

## References Cited

## UNITED STATES PATENTS

|           |        |               |          |
|-----------|--------|---------------|----------|
| 2,294,804 | 9/1942 | Ricketts      | 252—42.1 |
| 2,872,417 | 2/1959 | Jordan et al. | 252—42.1 |
| 2,929,785 | 3/1960 | Morway et al. | 252—41   |
| 2,999,066 | 9/1961 | Liddy         | 252—39   |

## FOREIGN PATENTS

|           |        |                |
|-----------|--------|----------------|
| 1,036,692 | 7/1966 | Great Britain. |
|-----------|--------|----------------|

## OTHER REFERENCES

"Extreme Pressure Lubricants," by Davey, in Industrial and Engineering Chem., September 1950, pp. 1841-1847.

DANIEL E. WYMAN, Primary Examiner

I. VAUGHN, Assistant Examiner